# EUROPEAN PATENT SPECIFICATION

(11) **EP 1 143 024 B1**
(45) Date of publication and mention of the grant of the patent: **30.11.2005**
(21) Application number: 99959849.3
(22) Date of filing: 16.12.1999
(51) Int. Cl.: C22C 38/00, C22C 38/44, C22C 38/50, C22C 38/42, C22C 38/48

(54) **MARTENSITIC STAINLESS STEEL**
MARTENSITISCHER, ROSTFREIER STAHL
ACIER INOXYDABLE MARTENSITIQUE

(30) Priority: 18.12.1998 JP 36049398
(43) Date of publication of application: 10.10.2001
(73) Proprietor: JFE Steel Corporation, Tokyo, 100-0011 (JP)
(72) Inventor: MINAMI, Yusuke, Tokyo 100-0005 (JP); MASAMURA, Katsumi, Tokyo 100-0005 (JP); SUZUKI, Toshio, Tokyo 100-0005 (JP)
(74) Representative: HOFFMANN EITLE
(86) International application number: PCT/JP1999/007067
(87) International publication number: WO 2000/037700

(56) References cited:
- EP-A- 0 565 117
- EP-A- 0 649 915
- EP-A1- 0 798 394
- WO-A-96/03532
- JP-A- 7 310 143
- JP-A- 8 041 599
- JP-A- 9 125 141
- JP-A- 9 327 721
- JP-A- 10 204 587
- PATENT ABSTRACTS OF JAPAN vol. 1998, no. 03, 27 February 1998 (1998-02-27) -& JP 09 291344 A (NIPPON STEEL CORP), 11 November 1997 (1997-11-11)
- PATENT ABSTRACTS OF JAPAN vol. 1996, no. 06, 28 June 1996 (1996-06-28) -& JP 08 041599 A (SUMITOMO METAL IND LTD), 13 February 1996 (1996-02-13)
- PATENT ABSTRACTS OF JAPAN vol. 1998, no. 05, 30 April 1998 (1998-04-30) -& JP 10 025549 A (NIPPON STEEL CORP), 27 January 1998 (1998-01-27)
- PATENT ABSTRACTS OF JAPAN vol. 017, no. 554 (C-1118), 6 October 1993 (1993-10-06) -& JP 05 156409 A (NIPPON STEEL CORP), 22 June 1993 (1993-06-22)
- PATENT ABSTRACTS OF JAPAN vol. 015, no. 317 (C-0858), 13 August 1991 (1991-08-13) -& JP 03 120337 A (SUMITOMO METAL IND LTD), 22 May 1991 (1991-05-22)

## Description

### Field of the Invention

The present invention relates to a martensitic stainless steel suitable for pipelines or the like which are used under environments containing both moist carbon dioxide gas and moist hydrogen sulfide.

### Description of the Prior Art

Steels for pipelines transporting oil and natural gas are requested to have excellent corrosion resistance and field welding performance responding to each use environment. In this respect, carbon steel pipes of X50 and X65 grades have often been adopted. The term "excellent field welding performance" referred to herein signifies the welding not requiring preheating and postheating that are applied to prevent welding crack generation observed during field welding of pipelines.

In recent years, environments containing moist carbon dioxide gas and moist hydrogen sulfide have increased, and the application of stainless steels are studied from the standpoint of corrosion resistance. Existing stainless steels, however, did not necessarily have sufficient performance for pipelines. Consequently, stainless steels such as those containing 0.2%C-13%Cr and two-phase stainless steels such as those containing 22%Cr and 25%Cr were developed. The former 0.2%C-13%Cr stainless steel was developed for oil well use that does not require welding. Therefore, the 0.2%-13%Cr stainless steel is not suitable for the pipelines that need excellent field welding performance because the welding needs preheating and postheating at high temperatures to prevent weld crack generation. The latter two-phase stainless steel containing 22%Cr or 25%Cr does not need preheating and postheating on welding. However, the two-phase stainless steel is difficult in use as pipelines that need a large quantity of steels because the stainless steel is expensive.

To cope with the situation, stainless steel containing less C and containing 13%Cr is proposed in JP-A-6-100943, (the term "JP-A-" referred to herein signifies "Unexamined Japanese Patent Publication"), JP-A-4-268018, JP-A-8-100235, and JP-A-8-100236. Other martensitic stainless steels with low C content and Mo content around 2.0 but with no W are described in JP-A-9-291344, JP-A-8-41599, WO 96/03532 and JP-A-10-25549, However, that type of stainless steel cannot satisfy simultaneously the requirement of corrosion resistance to an environment containing both moist carbon dioxide gas and moist hydrogen sulfide and the requirement of field welding performance.

WO 96/21747 on the other hand proposes martensitic stainless steels containing Mo or Mo and W but having a much larger content of C (0.15-0.40 %). Hence these steels cannot be used for pipelines under moist carbon dioxide of hydrogen sulfide environments as Mo and W are strong carbide former elements.

### Summary of the Invention

An object of the present invention is to provide a martensitic stainless steel applicable under environments containing both moist carbon dioxide gas and moist hydrogen sulfide, and having excellent field welding performance.

To attain the object, the inventors of the present invention carried out various investigations on the components of martensitic stainless steel, and obtained the following-given findings
- Chromium is effective in corrosion resistance to an acid in a moist carbon dioxide gas.
- To prevent occurrence of sulfide stress corrosion cracking in an environment containing moist hydrogen sulfide, the suppression of quantity of invading hydrogen into the steel is required. To do this, it is effective to add a certain amount of Mo along with Cr, and further to reduce the amount of desulfurization and deoxidization elements.
- Control of C and N amount is effective to improve the welding and production performance.
- Tungsten reveals a remarkable increase in proof stress and excellent corrosion resistance in moist carbon dioxide gas.

Based on the findings, the inventors of the present invention have developed a martensitic stainless steel consisting of 0.02% or less C, 0.02% or less N, 0.1 to 0.3% Si, 0.1 to 0.3% Mn, 10 to 13% Cr, 5 to 8% Ni, 1.5 to 3% Mo, 0.1 to 3% W, further optionally one or both of 0.01 to 0.1% Ti and Nb, and optionally 0.1 to 3% Cu, by weight, and the balance of Fe and inevitable impurities, and satisfying 0.02 to 0.04% (C + N) by weight.

The object of the present invention can be achieved also by a martensitic stainless steel consisting of 0.02% or less C, 0.02% or less N, 0.1 to 0.3% Si, 0.1 to 0.3% Mn, 10 to 13% Cr, 5 to 8% Ni, 1.5 to 3% Mo, 0.1 to 3% W, further one or both of 0.01 to 0.1% Ti and Nb, and optionally 0.1 to 3% Cu, by weight, and the balance of Fe and inevitable impurities, and satisfying 0.02 to 0.04% (C + N) by weight.

### Best Mode to Carry Out the Invention

The reasons to limit the components of the martensitic stainless steels according to the present invention are described in the following.

### Carbon:

Carbon is an element to form a carbide combining with Cr, thus strengthening the steel. Carbon, however, reduces the amount of chromium which is effective in corrosion resistance and increases the hardness at a weld heat-affected zone (HAZ), thus requiring heat treatment after welding. Accordingly, the C content is specified to 0.02 wt.% or less.

### Nitrogen

Nitrogen combines with Cr to form a compound, thus reducing the amount of Cr which is effective in corrosion resistance, and increases the hardness at the HAZ. Consequently, the N content is specified to 0.02 wt.% or less.

### Silicon

Silicon is added as a deoxidizer. The Si content of not more than 0.1 wt.% gives no effect of deoxidization. The Si content of more than 0.3 wt.% induces crystallization of delta ferrite, then an additional Ni amount are needed to maintain the phase balance. Therefore, the Si content is specified to a range of from 0.1 to 0.3 wt.%.

### Manganese

Manganese is added as a desulfurizer. The Mn content of not more than 0.1 wt.% gives no effect of desulfurization, and degrades hot workability. The Mn content of more than 0.3 wt.% degrades the corrosion resistance under an environment containing carbon dioxide and hydrogen sulfide. Accordingly, the Mn content is specified to a range of from 0.1 to 0.3 wt.%.

### Chromium

Chromium is an element which is effective to improve the corrosion resistance under an environment containing moist carbon dioxide gas. However, less than 10 wt.% of Cr content cannot attain the effect. With the increase in the Cr content, the corrosion resistance increases. Since Cr is a powerful element to produce ferrite, if the Cr content exceeds 13 wt.%, surplus addition of Ni which is an expensive element to produce austenite is required. Consequently, the Cr content is specified to a range of from 10 to 13 wt.%.

### Nickel

Although Ni is an element necessary to form a martensitic structure, less than 5 wt.% of Ni content degrades toughness and corrosion resistance owing to generating a large quantity of ferritic phase. If the Ni content exceeds 8 wt.%, the economy degrades. Therefore, the Ni content is specified to a range of from 5 to 8 wt.%.

### Molybdenum

Molybdenum is an effective element to attain corrosion resistance. However, less than 1.5 wt.% of Mo content gives insufficient effect. If Mo is added over 3 wt.%, addition of expensive Ni is required because Mo is an element to generate ferrite.

Adding to the above-described specification of each element, it is required that the amount of (C + N) is 0.02 wt.% or more to attain an aimed strength, and is not more than 0.04 wt.% to control the hardness at the HAZ.

### Tungsten and copper

Each of W and Cu is an element effective to attain strength and corrosion resistance. Addition of W or Cu to less than 0.1 wt.% does not attain sufficient effect, and, to over 3 wt.% degrades the hot workability. Accordingly, the content of W and Cu is specified to a range of from 0.1 to 3 wt.%.

### Titanium and niobium

Each of Ti and Nb forms a carbide with C in steel, and refines grains to improve the strength and toughness. Addition of Ti or Nb to less than 0.01 wt.% does not attain sufficient effect, and, to over 0.1 wt.% saturates the effect. Consequently, the content of Ti and Nb is specified to a range of from 0.01 to 0.1 wt.%.

The steels with the components adjusted as described above according to the present invention are stable in their mechanical characteristics against variations of production conditions such as heat treatment.

The steels according to the present invention may be prepared by melting using adequate methods such as converter, electric furnace, or combination of them, if only the components thereof are adjusted to a specified range. After prepared by melting, the steels are formed in billets and slabs by a continuous casting machine or a mold, then are worked into a specified shape such as steel pipes and steel plates by hot-rolling, followed by applying heat treatment to attain an aimed strength. After established a martensitic structure by a heat treatment, the steels are preferred to be subjected to a tempering to adjust the strength thereof.

### Example 1

Steels A through Q having respective chemical compositions given in Table 1 were prepared by melting in a vacuum melting furnace. Each of the steels was hot-rolled to a steel plate having 12 mm in thickness. The steel plate was quenched by water from 900°C ± 10°C, and then tempered at 640°C ± 5°C to obtain aimed proof stresses of from 600 to 700 MPa. For each of thus prepared steel plates, the corrosion resistance and the field welding performance described below were tested.

The corrosion resistance to a moist carbon dioxide gas was evaluated in terms of plate thickness loss by immersing a steel plate in a solution of 5% NaCl-30atmCO₂ at 180°C for 96 hours. If the corrosion rate converted to one-year value is not more than 0.3 mm/y, no practical application problem occurs.

The corrosion resistance to a moist hydrogen sulfide was evaluated in terms of presence/absence of fracture on the steel plate by the stress corrosion crack test for a sulfide, (Resistant SSC test) of TM0177 specified by NACE. That is, a steel plate was immersed in an aqueous solution of 5%NaCl+0.5%acetic acid saturated with 1atmH₂S for 720 hours while applying a load of 60% of the proof stress. If no fracture occurs under the test, no practical application problem occurs.

The field welding performance was evaluated by the hardness at a reproduced HAZ section. If the hardness is not more than 350 Hv, no preheating and postheating treatment are required.

Table 2 shows the results of the investigation.

The steels C, G, H and J, which are the Example Steels according to the present invention, gave 600 to 700 MPa of proof stress, 0.3 mm/y or less of corrosion rate in a moist carbon dioxide gas, and 350 Hv or less of hardness, giving no fracture in a moist hydrogen sulfide, being applicable in an environment containing both a moist carbon dioxide gas and a moist hydrogen sulfide, giving excellent field welding performance, thus showing adaptability to pipelines.

On the other hand, the Comparative Steel K contained less amount of Cr content and showed no sufficient corrosion resistance to a moist carbon dioxide. The Comparative Steel L contained large amount of Si which is a deoxidizer, the Comparative Steel M contained large amount of Mn as a desulfurizer, and the Comparative Steel N contained less amount of Mo, so that these comparative steels were inferior in corrosion resistance to a moist hydrogen sulfide. The Comparative Steel O contained less amount of Ni, so a delta ferrite deposited, which degraded the corrosion resistance to a moist carbon dioxide gas. The Comparative Steel P contained less amount of (C + N), and failed to attain satisfactory strength. The Comparative Example Q contained large amount of C and N, so that the strength was high and that the field welding performance was inferior.

**Table 2**

| Steel | Proof stress (MPa) | Corrosion in a moist carbon dioxide gas (mm/y) | Presence/absence of fracture in a moist hydrogen sulfide gas | Hardness (Hv) | Remark |
|---|---|---|---|---|---|
| A | 625 | 0.11 | Absent | 315 | Reference Steel |
| B | 690 | 0.15 | Absent | 316 | Reference Steel |
| C | 684 | 0.08 | Absent | 314 | Example Steel |
| D | 630 | 0.05 | Absent | 320 | Reference Steel |
| E | 622 | 0.14 | Absent | 310 | Reference Steel |
| F | 625 | 0.20 | Absent | 320 | Reference Steel |
| G | 644 | 0.12 | Absent | 318 | Example Steel |
| H | 651 | 0.18 | Absent | 315 | Example Steel |
| I | 614 | 0.22 | Absent | 314 | Reference Steel |
| J | 660 | 0.15 | Absent | 325 | Example Steel |
| K | 602 | 0.75 | Absent | 321 | Comparative Example Steel |
| L | 622 | 0.15 | Present | 313 | Comparative Example Steel |
| M | 618 | 0.14 | Present | 315 | Comparative Example Steel |
| N | 613 | 0.21 | Present | 312 | Comparative Example Steel |
| O | 656 | 0.42 | Absent | 309 | Comparative Example Steel |
| P | 575 | 0.16 | Absent | 297 | Comparative Example Steel |
| Q | 720 | 0.23 | Absent | 380 | Comparative Example Steel |

## Claims

1. A martensitic stainless steel consisting of 0.02% or less C, 0.02% or less N, 0.1 to 0.3% Si, 0.1 to 0.3% Mn, 10 to 13% Cr, 5 to 8% Ni, 1.5 to 3% Mo, 0.1 to 3% W, further optionally one or both of 0.01 to 0.1% Ti and Nb, and optionally 0.1 to 3% Cu, by weight, and the balance of Fe and inevitable impurities, and satisfying 0.02 to 0.04% (C + N) by weight.

2. A martensitic stainless steel according to claim 1, consisting of 0.02% or less C, 0.02% or less N, 0.1 to 0.3% Si, 0.1 to 0.3% Mn, 10 to 13% Cr, 5 to 8% Ni, 1.5 to 3% Mo, 0.1 to 3% W, further one or both of 0.01 to 0.1% Ti and Nb, and optionally 0.1 to 3% Cu, by weight, and the balance of Fe and inevitable impurities, and satisfying 0.02 to 0.04% (C + N) by weight.

## Patentansprüche

1. Martensitischer rostfreier Stahl, bestehend aus 0,02 % oder weniger C, 0,02 % oder weniger N, 0,1 bis 0,3 % Si, 0,1 bis 0,3 % Mn, 10 bis 13 % Cr, 5 bis 8 % Ni, 1,5 bis 3 % Mo, 0,1 bis 3 % W, ferner gegebenenfalls einem oder beiden von 0,01 bis 0,1 % Ti und Nb, und gegebenenfalls 0,1 bis 3 % Cu, pro Gewicht, und einem Rest aus Fe und unvermeidbaren Verunreinigungen, der 0,02 bis 0,04 % (C + N) pro Gewicht genügt.

2. Martensitischer rostfreier Stahl gemäss Anspruch 1, bestehend aus 0,02 % oder weniger C, 0,02 % oder weniger N, 0,1 bis 0,3 % Si, 0,1 bis 0,3 % Mn, 10 bis 13 % Cr, 5 bis 8 % Ni, 1,5 bis 3 % Mo, 0,1 bis 3 % W, ferner einem oder beiden von 0,01 bis 0,1 % Ti und Nb, und gegebenenfalls 0,1 bis 3 % Cu, pro Gewicht, und einem Rest aus Fe und unvermeidbaren Verunreinigungen, der 0,02 bis 0,04 % (C + N) pro Gewicht genügt.

## Revendications

1. Acier martensite inoxydable consistant en 0,02 % ou moins de C, 0,02% ou moins de N, 0,1 à 0,3% de Si, 0,1 à 0,3% de Mn, 10 à 13% de Cr, 5 à 8% de Ni, 1,5 à 3% de Mo, 0,1 à 3 % de W, de plus facultativement l'un ou les deux de 0,01 à 0,1 % de Ti et Nb, et facultativement de 0,1 à 3% en poids de Cu, en poids, et le reste de Fe et d'impuretés inévitables et satisfaisant à 0,02 à 0,04% en poids de (C + N).

2. Acier martensite inoxydable selon la revendication 1, consistant en 0,02% ou moins de C, 0,02 % ou moins de N, 0,1 à 0,3% de Si, 0,1 à 0,3% de Mn, 10 à 13% de Cr, 5 à 8% de Ni, 1,5 à 3% de Mo, 0,1 à 3% de W, de plus l'un ou les deux de 0,01 à 0,1% de Ti et Nb, et facultativement 0,1 à 3% de Cu, en poids, et le reste de Fe et d'impuretés inévitables, et satisfaisant à 0,02 à 0,04 % en poids de (C + N).
